

O. P. M. GOSS.  
ART OF PRESERVING WOOD.  
APPLICATION FILED NOV. 9, 1916.

1,252,428.

Patented Jan. 8, 1918.



Fig. 1.



Fig. 2.

INVENTOR  
Oliver P. M. Goss  
BY *Z. J. Geisler*  
ATTORNEY

# UNITED STATES PATENT OFFICE.

OLIVER P. M. GOSS, OF SEATTLE, WASHINGTON.

## ART OF PRESERVING WOOD.

1,252,428.

Specification of Letters Patent.

Patented Jan. 8, 1918.

Application filed November 9, 1916. Serial No. 130,461.

*To all whom it may concern:*

Be it known that I, OLIVER P. M. Goss, a citizen of the United States, and a resident of Seattle, King county, State of Washington, have invented a certain new and useful Improvement in the Art of Preserving Wood, of which the following is a specification.

In the preservative treatment of timber two methods are generally employed, namely, the timber may be immersed in the preserving fluid in an open tank, or under pressure; the latter being the method more generally used, since some timber, notably Douglas fir, resists the penetration of the preserving fluid to too great a degree across the grain, in an open tank, for such treatment to be practicable. The pressure method is, however, wasteful and unreliable, in fact deceptive, because while a given quantity of the preserving fluid may be driven into the pores of the timber, it is found that the larger portion of the fluid wastefully collects in certain areas while other areas are left practically without any. For this reason it is preferred to use the so-called perforation method, which consists in putting a number of holes into the outer surface of the wood and causing the preservative to enter the pores through such holes. In this way there is assured a definite degree of penetration, and a wider distribution of the preservative. But the latter method was also inefficient, for the holes or perforations above referred to were put into the timber more or less at random, that is, without regard to the normal, minimum spread of the preservative and the result was certain parts of the timber received an excess of the preservative while other parts receive an insufficient treatment. Another objection to said haphazard system of perforating the timber lies in the fact that it frequently results in the putting of a great number of perforations in one plane of cross section of the timber, and hence the transverse strength of the timber at that plane of cross section is materially reduced.

With the object of overcoming the above objections, and also for the purpose of providing a very simple and economical way of treating timber with a preservative fluid, to any desired degree of impregnation, and also insuring a substantially uniform impregnation of the surface treated by means of a minimum perforation of the timber,

I have invented the following method: The outer surface is perforated to a desired depth by holes systematically located at relative distances apart, both transversely and longitudinally, that is, with the grain of the wood and crosswise thereof, as predetermined by the known normal spread, that is, absorption, of the preservative with and across the grain of the wood under given factors of time of immersion, pressure applied and size of perforations. The result of such procedure is a substantially uniform treatment of the timber to a depth equal to that of the perforations, and without waste of the preservative.

In order to prevent a decrease in the transverse strength of the timber by the perforations put into the wood, I arrange the perforations in a series of planes lying diagonally with the grain of the wood. This, together with the other above mentioned features of my invention, can better be understood by having reference to the accompanying drawings, in which:

Figure 1 is a diagrammatic, sectional view of a block of timber representing a portion thereof as partially treated by my improved method, and shows the arrangement of the perforations with respect to the grain of the wood, and also represents the trend of the distribution of a preservative fluid from the perforations both in directions running with the grain and crosswise thereof; and

Fig. 2 is a section of the treated timber taken parallel with the bore of the perforations.

*a* represents a block of timber; *b* is the grain in same; *c* are the perforations through which a preservative fluid, such, for example, as creosote oil, is introduced into the timber; and *d* represents diagrammatically the areas over which the preservative spreads from each hole.

As is commonly known, the extent of absorption of a fluid will be much greater along the grain of the wood than across the same. The normal, minimum extent of the absorption, both with and across the grain of any given kind of timber, is readily determined by experiment for any particular length of time of immersion of the material in the preservative, pressure applied, and size of the perforations, and the same is then to be noted, and later, in practising my art, the perforations are to be made spaced apart accordingly. Furthermore, these per-

forations are to be relatively so located that the margins of the previously ascertained, and therefore known, minimum areas impregnated from the perforations will overlap at their margins.

By the staggering of the perforations, as shown in Fig. 1, the uniform and even treatment of the timber by the preservative is promoted without danger of the perforations being located so closely together as to appreciably reduce the transverse strength of the timber. Figs. 1 and 2 show views of timber in the process of being treated, but the adjacent treated areas have not yet come together and overlapped, as will be the case when the preservative has been fully absorbed by the timber.

I have tried out my invention in connection with both of the above named two general methods of treatment, and obtained these results:

By open tank method, in treating air-seasoned Douglas fir, previously perforated by small holes one-sixteenth of an inch in diameter and spaced four inches apart along the grain, and one-eighth inch apart across the grain, I obtained complete and substantially uniform penetration. The method of procedure resulting in this complete penetration, to the full depth of the perforation, was as follows: The timber was placed in the open tank and the preservative oil was introduced. The timber was boiled in the oil for four hours at 215 deg. Fahrenheit. The heat was then discontinued and the material allowed to cool down in the oil, which required a period of approximately twelve hours, after which the timber may be removed and is ready for use.

My second test was made under the pressure method. Complete penetration was secured the full depth of the perforations, the procedure being as follows: Air-seasoned

Douglas fir specimens were perforated to a depth of three-fourths of an inch by a tool 45 one-eighth inch in width across the grain. The spacing of the holes from each other along the grain was seven inches, and the spacing across the grain was three-eighths of an inch. The timbers perforated as herein 50 described were placed in a pressure retort, and preservative oil was introduced and raised to a temperature of 170 degrees Fahrenheit. The material was subjected to this temperature for four hours, after which 55 pressure was applied to the oil, varying from 0 to 120 pounds per square inch. About one hour was required to raise the pressure to 120 pounds. And it was held at this pressure for a period of two hours. During the pressure the temperature of the oil was 170 degrees 60 Fahrenheit.

After such treatment the timber is ready for use.

I claim:

1. The method of preparing a piece of wood for impregnation which comprises placing in a surface of the piece equally spaced rows of equally spaced holes so arranged that the distances between adjacent 70 holes are proportional to the rates of spread of the impregnating fluid in the directions in which the distances are measured.
2. The method of preparing a piece of wood for impregnation which comprises 75 placing in a surface of the piece equally spaced rows of equally spaced holes, so arranged that no row of holes extends in a direction directly across the grain of the piece, and arranged so that the distances between 80 adjacent holes are proportional to the rates of spread of the impregnating fluid in the directions in which the distances are measured.

O. P. M. GOSS.